# EUROPEAN PATENT SPECIFICATION

(11) **EP 3 797 898 B1**
(45) Date of publication and mention of the grant of the patent: **27.07.2022**
(21) Application number: 19199984.6
(22) Date of filing: 26.09.2019
(51) Int. Cl.: B22D 11/108, C21C 7/00

(54) **A MOULD FLUX AND THE USE THEREOF**
FORMFLUSSMITTEL UND VERWENDUNG DAVON
FLUX DE MOULAGE ET SON UTILISATION

(43) Date of publication of application: 31.03.2021
(73) Proprietor: AB Sandvik Materials Technology, 811 81 Sandviken (SE)
(72) Inventor: WALDÈN, Bertil, 811 61 Sandviken (SE); Paliwal, Manas, 411014 Pune (IN)
(74) Representative: Setréus, Ellen

(56) References cited:
- EP-A1- 3 372 325
- WO-A1-2007/148939
- DE-A1- 2 346 778
- JP-A- H04 138 857
- JP-A- 2012 066 304
- KR-A- 20190 097 901
- K.C. MILLS, A.B. FOX, R.P. THACKRAY, Z. LI: "The performance and properties of mould fluxes", PROC. VII INTERNATIONAL CONFERENCE ON MOLTEN SLAGS, FLUXES AND SALTS, 2004, XP002796638,

## Description

### TECHNICAL FIELD

The present disclosure relates to a mould flux and to a method of manufacturing a nickel-base alloy.

### BACKGROUND

When manufacturing nickel-base alloys, especially nickel-base alloys containing titanium, a problem has been noticed in connection to the Vacuum Arc Re-melting process (VAR) following the moulding of a piece of the alloy. as it has been seen that the arc may become unstable and, as a result thereof, the process sometimes stops. Such unwanted stops of the process are caused by the fact that a portion in the moulded piece has a substantially lower electric conductivity than the rest of the moulded piece, resulting in an unstable arc or extinction of the arc. It is therefore an aspect of the present disclosure to provide a solution or at least reduce the above-mentioned problem. KR2019009901 relates to a flux to be employed by casting of steels, said flux comprising SiO₂ 37.6-39.6 wt%, CaO 27.2-29.2 wt %, MgO 2.6-3.6 wt%, Al₂O₃1-3 wt %, Na₂O 15.1-16.1 wt%, K₂O 0.16-0.18 wt%, Fe₂O₃ 0.56-0.83 wt%, Li₂O 2.57-2.85 wt%.

### SUMMARY

The present disclosure therefore provides a mould flux having a composition of, in weight%

| | |
|---|---|
| SiO₂ | 15-25; |
| CaO | 15-35; |
| Al₂O₃ | 1-7; |
| Na₂O | 18-30; |
| K₂O | 15-25; |
| Fe₂O₃ | 0-5; |
| C | 0-4; |
| TiO₂ | 0-2; |
| MnO | 0-2; |
| MgO | 0-2; |
| Li₂O | 0-10; |

and wherein the melting point of the mould flux is less than or equal to 1300°C.

Mould fluxes are synthetic slags constituted by a complex mix of oxides, minerals and carbonaceous materials. The main oxides are silica (SiO₂), calcium oxide (CaO), sodium oxide (Na₂O), alumina (Al₂O₃) and magnesium oxide (MgO).

The liquid slag formed by the flux constitutes a barrier to avoid steel re-oxidation by contact with air and the entrapment of other gases, such as nitrogen. The fluxes can be added through the top of the mould on the liquid steel, manually or automatically.

According to one embodiment, the mould flux is provided as a powder having the above-mentioned or below-mentioned composition. The flux will then melt in contact with the molten alloy.

It has been found been surprisingly found that the use of the present mould flux when moulding Ni-base alloys, especially those nickel base alloys containing Ti will prevent or suppress the formation of portions of lower electric conductivity in the moulded piece, such that the above-mentioned problem during a subsequent VAR process is remedied.

When the nickel base alloy contains Ti, the presence of CaO in the mould flux and the Ti content in the nickel alloy will be responsible for the formation of Perovskite. Hence, the present composition limits the CaO content in the mould powder compared to conventional mould fluxes.

Additionally, if CaO content is lowered, then in order to control the various thermo-physical properties of mould powder such as melting point, density and viscosity, the content of SiO₂ should be lowered as well.

Furthermore, it has been found that local portions in moulded pieces of a Ni-base alloy, especially those containing titanium have a lower electric conductivity than the rest of the piece. This is due to the fact that said portions comprise a Perovskite phase. The Perovskite phase formation is assumed to be as follows: SiO₂+Ti→TiO₂+Si. As a result, TiO₂ may together with CaO form Perovskite as a solution of Ca₂Ti₂O₅ and Ca₂Ti₂O₆. As mentioned herein, CaO in the flux contributes to the formation of Perovskite. The mould flux according to the present disclosure suppresses the formation of a Perovskite phase compared to mould fluxes of prior art. A relatively low content of SiO₂ in the present mould flux powder and a relatively high content of alkali oxides (Na₂O and K₂O), and possibly also the effect of Li₂O and MgO, is assumed to suppress the formation of Perovskite.

According to one embodiment of the mould flux as defined hereinabove or hereinafter, at least a part of Na₂O, SiO₂ and Al₂O₃ present in the mould flux are in the form of Sodium Feldspar (Na_{0.33}Al_{0.35}Si_{1.13}O_{2.95}). According to further embodiments, at least 25%, or at least 40% of Na₂O, SiO₂ and Al₂O₃ present in the mould flux are in the form of Sodium Feldspar (Na_{0.33}Al_{0.35}Si_{1.13}O_{2.95}). According to further embodiments, at least 50%, or at least 90% of the Na₂O present in the mould flux is in the form of Sodium Feldspar, (Na_{0.33}Al_{0.35}Si_{1.13}O_{2.95}).

According to one embodiment of the mould flux as defined hereinabove or hereinafter, at least a part of K₂O, SiO₂ and Al₂O₃ present in the mould flux is present in the form of Potassium Feldspar (K_{0.33}Al_{0.35}Si_{1.13}O_{2.95}). According to further embodiments at least 25%, or at least 40% of K₂O, SiO₂ and Al₂O₃ present in the mould flux is present in the form of Potassium Feldspar (K_{0.33}Al_{0.35}Si_{1.13}O_{2.95}). According to further embodiments, at least 50%, or at least 90%, of the K₂O present in the mould flux is present in the form of Potassium Feldspar (K_{0.33}Al_{0.35}Si_{1.13}O_{2.95}).

According to one embodiment, the content of Na₂O in the mould flux is 18-25 weight%.

According to one embodiment, the content of K₂O in the mould flux is 15-22 weight%.

According to one embodiment, the content of TiO₂ in the mould flux is >0.05 weight%.

According to one embodiment, the content of Li₂O in the mould flux is >1.0 weight%.

According to one embodiment, the ratio of SiO₂/(CaO+Al₂O₃)>1 .

According to one embodiment, the ratio of CaO and SiO₂ (CaO/SiO₂)- is in the range of 3:4 to 4:3, such as 1:1. These oxides are important to control the viscosity and the melting point of the mould flux. A CaO content greater than 35 weight% will promote the formation of Perovskite and CaO less than 15 % might induce high viscosity in the molten mould powder. The content of SiO₂ should be controlled on the basis of CaO.

Na₂O, K₂O and Li₂O will stabilize Ti in the melt and thereby as mentioned above will contribute to the prevention of Perovskite formation. This is best results are achieved when each of Na₂O and K₂O is present in an amount of 18-22 weight%, preferably around 20 weight%, in the mould mixture. In addition, these alkali oxides promote the formation of Nepheline phase which is beneficial during casting. A very high content of these oxides will make the flux mould too fluid and a too low content would result in formation of Perovskite phase.

The objective of the present disclosure is also achieved by means of a method of moulding a piece of a Ni-base alloy wherein a mould flux as defined hereinabove or hereinafter is applied on a surface of the molten alloy during moulding thereof.

According to one embodiment, the Ni-base alloy comprises, in weight%:

| | |
|---|---|
| C | <0.05; |
| Cr | 17-23; |
| Ni | 35-63; |
| Mo | 2.5-9.5; |
| Ti | 0.3-3.0; |
| Al | 0-0.7; |
| Si | 0-0.5; |
| Nb | 0-4.5; |
| Cu | 0-3; |
| Mn | 0-0.1; |
| S | 0-0.003; |
| P: | 0-0.02; |

balance Fe.

## Claims

1. A mould flux having a composition of, in weight%:
| | |
|---|---|
| SiO₂ | 15-25; |
| CaO | 15-35; |
| Al₂O₃ | 1-7; |
| Na₂O | 18-30; |
| K₂O | 15-25; |
| Fe₂O₃ | 0-5; |
| C | 0-4; |
| TiO₂ | 0-2; |
| MnO | 0-2; |
| MgO | 0-2; |
| Li₂O | 0-10; |
and wherein the melting point of the mould flux is less than or equal to 1300°C.

2. The mould flux according to claim 1, wherein at least a part of Na₂O, SiO₂ and Al₂O₃ present in the mould flux is present in the form of Sodium Feldspar, Na_{0.33}Al_{0.35}Si_{1.13}O_{2.95}.

3. The mould flux according to claim 1 or 2, wherein at least a part of K₂O, SiO₂ and Al₂O₃ present in the mould flux is present in the form of Potassium Feldspar, K_{0.33}Al_{0.35}Si_{1.13}O_{2.95}.

4. The mould flux according to any one of claims 1-3, wherein at least 50% of the Na₂O present in the mould flux is in the form of Sodium Feldspar, Na_{0.33}Al_{0.35}Si_{1.13}O_{2.95}.

5. The mould flux according to any one of claims 1-4, wherein at least 50%, of the K₂O present in the mould flux is present in the form of Potassium Feldspar, K_{0.33}Al_{0.35}Si_{1.13}O_{2.95}.

6. The mould flux according to any one of claims 1-5, wherein the content of Na₂O, in weight%, is 18-25.

7. The mould flux according to any one of claims 1-6, wherein the content of K₂O, in weight %, is 15-22.

8. The mould flux according to any one of claims 1-7, wherein the content of TiO₂ is >0.05 weight%.

9. The mould flux according to any one of claims 1-8, wherein the content of Li₂O is >1.0 weight%.

10. The mould flux according to any one of claims 1-9, wherein SiO₂/(CaO+Al₂O₃)>1.

11. The mould flux according to any one of claims 1-10, wherein the ratio between CaO and SiO₂ is in the range of 3:4 - 4:3.

12. The mould flux according to any one of claims 1-11, wherein the mould flux is a powder having the composition according to any one of claims 1-11.

13. A method of manufacturing a nickel-base alloy, wherein a mould flux according to any one of claims 1-12 is applied on a surface of the molten nickel-base alloy during moulding thereof.

14. A method according to claim 13, wherein said Ni-base alloy comprises, in weight%:
| | |
|---|---|
| C | <0.05; |
| Cr | 17-23; |
| Ni | 35-63; |
| Mo | 2.5-9.5; |
| Ti | 0.3-3.0; |
| Al | 0-0.7; |
| Si | 0-0.5; |
| Nb | 0-4.5; |
| Cu | 0-3; |
| Mn | 0-0.1; |
| S | 0-0.003; |
| P: | 0-0.02; |
balance Fe.

## Patentansprüche

1. Formflussmittel, das in Gewichts-% eine Zusammensetzung wie folgt aufweist:
| | |
|---|---|
| SiO₂ | 15 - 25; |
| CaO | 15 - 35; |
| Al₂O₃ | 1 - 7; |
| Na₂O | 18 - 30; |
| K₂O | 15 - 25; |
| Fe₂O₃ | 0 - 5; |
| C | 0 - 4; |
| TiO₂ | 0 - 2; |
| MnO | 0-2; |
| MgO | 0-2; |
| Li₂O | 0 -10; |
und wobei der Schmelzpunkt des Formflussmittels niedriger oder gleich 1300 °C ist.

2. Formflussmittel nach Anspruch 1, wobei mindestens ein Teil von in dem Formflussmittel vorhandenen Na₂O, SiO₂ und Al₂O₃ in der Form von Natriumfeldspat, Na_{0,33}Al_{0,35}Si_{1,13}O_{3,95}, vorhanden ist.

3. Formflussmittel nach Anspruch 1 oder 2, wobei mindestens ein Teil von in dem Formflussmittel vorhandenen K₂O, SiO₂ und Al₂O₃ in der Form von Kaliumfeldspat, K_{0,33}Al_{0,35}Si_{1,13}O_{2,95}, vorhanden ist.

4. Formflussmittel nach einem der Ansprüche 1 - 3, wobei mindestens 50 % des in dem Formflussmittel vorhandenen Na₂O in der Form von Natriumfeldspat, Na_{0,33}Al_{0,35}Si_{1,13}O_{2,95}, ist.

5. Formflussmittel nach einem der Ansprüche 1 - 4, wobei mindestens 50 % des in dem Formflussmittel vorhandenen K₂O in der Form von Kaliumfeldspat, K_{0,33}Al_{0,35}Si_{1,13}O_{2,95}, vorhanden ist.

6. Formflussmittel nach einem der Ansprüche 1 - 5, wobei der Gehalt an Na₂O in Gewichts-% 18 - 25 beträgt.

7. Formflussmittel nach einem der Ansprüche 1 - 6, wobei der Gehalt an K₂O in Gewichts-% 15 - 22 beträgt..

8. Formflussmittel nach einem der Ansprüche 1 - 7, wobei der Gehalt an TiO₂ > 0,05 Gewichts-% beträgt.

9. Formflussmittel nach einem der Ansprüche 1 - 8, wobei der Gehalt an Li₂O > 1,0 Gewichts-% beträgt.

10. Formflussmittel nach einem der Ansprüche 1 - 9, wobei SiO₂/(CaO+Al₂O₃) > 1.

11. Formflussmittel nach einem der Ansprüche 1 - 10, wobei das Verhältnis zwischen CaO und SiO₂ im Bereich von 3:4 - 4:3 liegt.

12. Formflussmittel nach einem der Ansprüche 1-11, wobei das Formflussmittel ein Pulver ist, das eine Zusammensetzung nach einem der Ansprüche 1-11 aufweist.

13. Verfahren zum Herstellen einer Nickelbasislegierung, wobei ein Formflussmittel nach einem der Ansprüche 1 - 12 auf eine Oberfläche der geschmolzenen Nickelbasislegierung während deren Formen angewendet wird.

14. Verfahren nach Anspruch 13, wobei die Ni - Basislegierung in Gewichts-% Folgendes umfasst:
| | |
|---|---|
| C | < 0,05; |
| Cr | 17 - 23; |
| Ni | 35 - 63; |
| Mo | 2,5 - 9,5; |
| Ti | 0,3 - 3,0; |
| Al | 0 - 0,7; |
| Si | 0 - 0,5; |
| Nb | 0-4,5; |
| Cu | 0 - 3; |
| Mn | 0-0,1; |
| S | 0 - 0,003; |
| P: | 0 - 0,02; |
Rest Fe.

## Revendications

1. Flux de moulage présentant une composition de, en % en poids :
| | |
|---|---|
| SiO₂ | 15-25 ; |
| CaO | 15-35; |
| Al₂O₃ | 1-7; |
| Na₂O | 18-30; |
| K₂O | 15-25 ; |
| Fe₂O₃ | 0-5 ; |
| C | 0-4 ; |
| TiO₂ | 0-2 ; |
| MnO | 0-2; |
| MgO | 0-2; |
| Li₂O | 0-10 ; |
et dans lequel le point de fusion du flux de moulage est inférieur ou égal à 1 300 °C.

2. Flux de moulage selon la revendication 1, dans lequel au moins une partie de Na₂O, SiO₂ et Al₂O₃ présents dans le flux de moulage est présente sous la forme de feldspath de sodium, Na_{0,33}Al_{0,35}Si_{1,13}O_{2,95}.

3. Flux de moulage selon la revendication 1 ou 2, dans lequel au moins une partie de K₂O, SiO₂ et Al₂O₃ présents dans le flux de moulage est présente sous la forme de feldspath de potassium, K_{0,33}Al_{0,33}Si_{1,13}O_{2,95}.

4. Flux de moulage selon l'une quelconque des revendications 1-3, dans lequel au moins 50 % du Na₂O présent dans le flux de moulage est sous la forme de feldspath de sodium, Na_{0,33}Al_{0,35}Si_{1,13}O_{2,95}.

5. Flux de moulage selon l'une quelconque des revendications 1-4, dans lequel au moins 50 %, du K₂O présent dans le flux de moulage est présent sous la forme de feldspath de potassium, K_{0,33}Al_{0,35}Si_{1,13}O_{2,95}.

6. Flux de moulage selon l'une quelconque des revendications 1-5, dans lequel la teneur en Na₂O, en % en poids, est 18-25.

7. Flux de moulage selon l'une quelconque des revendications 1-6, dans lequel la teneur en K₂O, en % en poids, est 15-22.

8. Flux de moulage selon l'une quelconque des revendications 1-7, dans lequel la teneur en TiO₂ > 0,05 % en poids.

9. Flux de moulage selon l'une quelconque des revendications 1-8, dans lequel la teneur en Li₂ > 0,05 % en poids.

10. Flux de moulage selon l'une quelconque des revendications 1-9, dans lequel SiO₂/(CaO+Al₂O₃) > 1.

11. Flux de moulage selon l'une quelconque des revendications 1-10, dans lequel le rapport entre CaO et SiO₂ est dans la plage de 3:4 - 4:3.

12. Flux de moulage selon l'une quelconque des revendications 1-11, dans lequel le flux de moulage est une poudre présentant la composition selon l'une quelconque des revendications 1-11.

13. Procédé de fabrication d'un alliage à base de nickel, dans lequel un flux de moulage selon l'une quelconque des revendications 1-12 est appliqué sur une surface de l'alliage à base de nickel fondu pendant son moulage.

14. Procédé selon la revendication 13, dans lequel ledit alliage à base de Ni comprend, en % en poids :
| | |
|---|---|
| C | < 0,05 ; |
| Cr | 17-23 ; |
| Ni | 35-63 ; |
| Mo | 2,5-9,5 ; |
| Ti | 0,3-3,0 ; |
| Al | 0-0,7 ; |
| Si | 0-0,5 ; |
| Nb | 0-4,5 ; |
| Cu | 0-3 ; |
| Mn | 0-0,1 ; |
| S | 0-0,003 ; |
| P : | 0-0,02 ; |
le reste du Fe.
